# EUROPEAN PATENT SPECIFICATION

(11) **EP 0 281 060 B1**
(45) Date of publication and mention of the grant of the patent: **02.06.1993**
(21) Application number: 88103032.4
(22) Date of filing: 01.03.1988
(51) Int. Cl.: C10M 169/04

(54) **Lubricating oil compositions for traction drive**
Schmiermittelzusammensetzungen für Reibungsdruckantrieb
Compositions d'huile lubrifiante pour mécanismes de traction

(30) Priority: 02.03.1987 JP 47398/87
(43) Date of publication of application: 07.09.1988
(73) Proprietor: IDEMITSU KOSAN COMPANY LIMITED, Tokyo 100 (JP)
(72) Inventor: Hata, Hitoshi, Sodegaura-machi Kimitsu-gun Chiba-ken (JP); Machida, Hisashi, Maebashi-shi Gunma-ken (JP)
(74) Representative: Türk, Gille, Hrabal, Leifert

(56) References cited:
- EP-A- 0 088 453
- EP-A- 0 208 541
- EP-A- 0 218 086
- EP-A- 0 220 426
- US-A- 3 657 369
- US-A- 3 843 537
- US-A- 3 903 001

## Description

### Field of the Invention

The present invention relates to a lubricating oil composition for traction drive and, more particularly, to a lubricating oil composition which has a high coefficient of traction, shows a limited change in the coefficient of traction at low temperatures, excels in wear resistance, load carrying capacity, thermal and oxidation stability and rust preventing property, and can effectively be used as the lubricating oil for power transmission systems including a traction drive mechanism.

### Statement of the Prior Art

In recent years, traction drives (friction driving device utilizing rolling contact) have been applied as the continuously variable transmission for automotive and industrial purposes. The fluids used for such traction drives are required to have a high coefficient of traction and excel in power transmission efficiency.

A number of proposals have been made of the traction drive fluids meeting such demands (for instance, JP-B-46-338, 46-339, 47-35763 and 58-27838). All these proposals have their objects to improve the coefficient of traction.

As a result of testing the performance of such fluids for traction drive with actual machines, however, it has been found that they are poor in power transmission ability at low temperatures, and are thus practically unsatisfactory.

In power transmission systems exposed to low to high temperature environments, the coefficient of traction of these fluids changes depending upon temperature and, in particular, drops remarkably at low temperatures. Thus, problems arise in connection with practical performance in winter and cold districts.

From EP-A-0 208 541 lubricant compositions for use in traction drives are known which incorporate a selected hydrocarbon type of base oils combined with specified amounts of selected zinc dialkyldithio phosphates, alkenyl succinimides or their boron derivatives, carboxylic acid esters of polyalcohols. Although these composition provide traction drive apparatus with prolonged fatigue life, high oxidation stability, high shear stability, high traction coefficient, high wear resistance and rust-proofness, they do no more meet the actuel still higher requirements.

### SUMMARY OF THE INVENTION

The object of the present invention is to provide a lubricating oil composition for traction drive, which has a still higher coefficient of traction, shows a limited change in the coefficient of traction at low temperatures, and excels in wear resistance, load carrying capacity, thermal and oxidation stability and rust preventing property.

This object according to the present invention is achieved by the provision of a lubricating oil composition for traction drive, which comprises:
(A) a base oil containing as the main component a saturated hydrocarbon or hydrocarbons having fused ring and/or nonfused ring,
(B) an ethylene-α-olefin copolymer having a number-average molecular weight of 800 to 8,000,
(C) an anti-wear agent, and
(D) a polymethacrylate having a number-average molecular weight of 10,000 to 100,000,
wherein the anti-wear agent is at least one selected from the group consisting of zinc dithiophosphate, oxymolybdenum organophosphorodithioate sulfide, phosphate, phosphite, amine salt of phosphate, amine salt of phosphite, molybdenum dialkyldithiocarbamate, mixtures of sulfurized fats and oils and posphates, mixtures of sulfurized fats and oils and phosphites, mixtures of sulfurized olefin and phosphates, mixtures of sulfurized olefin and phosphites, and the amine salts of the aforementioned mixtures.

Preferred embodiments of the claimed lubricating oil composition are described in the subclaims.

### BRIEF DESCRIPTION OF THE DRAWING

Figure 1 shows the coefficients of traction µ measured in Example 1 and in comparative examples 1 and 2.

### DETAILED DESCRIPTION OF PREFERRED EMBODIMENTS

In the present invention, a base oil containing as the main component a saturated hydrocarbon or hydrocarbons having fused ring and/or nonfused ring is used as the component (A).

Various saturated hydrocarbons may be used to this end. In particular, it is preferred to use saturated hydrocarbons containing cyclohexyl group and/or decalyl group, and saturated hydrocarbons of 10 to 40 carbon atoms. By way of example, the following saturated hydrocarbons containing cyclohexyl group and/or decalyl group may be used.
3-methyl-1,3-dicyclohexylbutane expressed by:
1-cyclohexyl-1-decalylethane expressed by:
2,4-dicyclohexylpentane expressed by:
2-methyl-2,4-dicyclohexylpentane expressed by:
Alkylcyclohexanes expressed by:
wherein R¹ stands for an alkyl group having 10 to 30 carbon atoms. By way of example, reference may be made to isododecylcyclohexane and isopentadecylcyclohexane.

Besides, the following saturated hydrocarbons having fused ring and/or nonfused ring may be used as the component (A) in the present invention.
1,2-di(dimethylcyclohexyl)propane expressed by:
2,3-di(methylcyclohexyl)-2-methylbutane expressed by:
1,2-di(methylcyclohexyl)-2-methylpropane expressed by:
2,4-dicyclohexylpentane expressed by:
Cyclohexylmethyldecalin expressed by:
1-(methyldecalyl)-1-cyclohexylethane expressed by:
and
1-(dimethyldecalyl)-1-cyclohexylethane expressed by:
and
2-decalyl-2-cyclohexylpropane expressed by:
Cyclohexylmethyl perhydrofluorene expressed by:
1-perhydrofluorenyl-1-cyclohexylethane expressed by:
Cyclohexylmethyl perhydroacenaphthene expressed by:
1,1,2-tricyclohexylethane expressed by:
Bis-decalin expressed by:
1,3,5-tricyclohexyl-5-methylhexane expressed by:
2-(2-decalyl)-2,4,6-trimethylnonane expressed by:
1,1-didecalylethane expressed by:
Tercyclohexyl expressed by:
1,1,3-trimethyl-3-cycloexylhydrindane expressed by:
2-methyl-1,2-didecalylpropane expressed by:
These hydrocarbons may be used alone or in combination of more than 2 kinds.

Among others, preference is given to 1-cyclohexyl-1-decalylethane expressed by:
Preferably, this hydrocarbon should contain the cis-type compound in a larger amount, inter alia, in an amount of 50% or higher.

In the present invention, the component (A) is a base oil composed mainly of the aforesaid saturated hydrocarbon or hydrocarbons having fused ring and/or a nonfused ring, which may further contain mineral oils, particularly naphthenic mineral oil and synthetic oils such as polybutene and alkylbenzene in proportions of up to 50%.

In the present invention, the component (B) used is an ethylene-α-olefin copolymer having a number-average molecular weight of 800 to 8,000, preferably 1000 to 5,000, and more preferably 2,000 to 4,000. Copolymers having a number-average molecular weight of below 800 and exceeding 8,000 are unpreferred, since the reduction in the coefficient of traction at low temperatures is increased. The ethylene-α-olefin copolymers should have a kinematic viscosity of 20 to 10 000 mm²/s (20 to 10,000 cSt), preferably 40 to 8 000 mm²/s (40 to 8,000 cSt) at 100°C. The ethylene-α-olefin copolymers are oligomers of ethylene with α-olefins having 3 to 20 carbon atoms, for instance, propylene, 1-butene and 1-decene, and are hydrocarbonic synthetic oils free from any polar group. The ethylene content of the copolymers should preferably be 30 to 80 mol %, preferably 50 to 80 mol %. The component (B) is used in a proportion of 1 to 20 weight %, preferably 2 to 10 weight % based on the total amount of the compositions. The proportions of the component (B) below 1 weight % and above 20 weight % are unpreferred, since the reduction in the coefficient of traction at low temperatures is increased.

For such ethylene-α-olefin copolymers, commercially available copolymers may be used. By way of example, Lucant HC10, HC20, HC40, HC100, HC150, HC600 and HC2000 (tradename; produced by Mitsui Petrochemical Co., Ltd.) may be used alone or in suitable combinations.

In the present invention, anti-wear agents are further used as the component (C).

The anti-wear agents used include zinc dithiophosphate, oxymolybdenum organophosphorodithioate sulfide, phosphoric and phosphorous compound such as, phosphate, phosphite and amine salts thereof, and molybdenum dialkyldithiocarbamate, as well as mixtures of sulfurized fats and oils and phosphates, mixtures of sulfurized fats and oils and phosphites, mixtures of sulfurized olefin and phosphates, mixtures of sulfurized olefin and phosphites, and the amine salts of the aforementioned mixtures known as sulfur-phosphor-based extreme pressure agent (SP-based extreme pressure agent).

The zinc dithiophosphates are expressed in terms of the following general formula:
wherein R², R³, R⁴ and R⁵ may be identical or different, and stand for a primary alkyl group having 3 to 30 carbon atoms, a secondary alkyl group having 3 to 30 carbon atoms or an alkyl group-substituted aryl group having 6 to 30 carbon atoms.

Various zinc dithiophosphates expressed in terms of the general formula [I], in which the substituents R² to R⁵ may be identical or different, may be used alone or in combinations. Usually, two or more zinc dithiophosphates, in which all the substituents R² to R⁵ are identical, are mixed together for use. However, such zinc dithiophosphates may be used alone. Zinc dithiophosphates, in which the substituents R² to R⁵ are different, may also be used alone or in a suitable combination with the zinc dithiophosphates in which R² to R⁵ are identical. However, it is noted that, in either case, the zinc dithiophosphate containing a primary alkyl group having 3 to 30 carbon atoms amounts to 1/3, particularly 1/2 (on the weight basis) of all the zinc dithiophosphates.

By using the zinc dithiophosphates in which the zinc dithiophosphate containing a primary alkyl group amounts to at least 1/3 of the total amount of R² to R⁵ in all the zinc dithiophosphates_{,} it is possible to improve further anti-wear property and load carrying capacity and extend fatigure life, thereby enhancing durability.

For such zinc dithiophosphates_{,} commercially available ones may be used. By way of example, Lubrizol 1097 (R² to R⁵ are mainly primary octyl groups), Lubrizol 1395 (R² to R⁵ are mainly primary butyl and amyl groups sold by Nippon Lubrizol Co.; OLOA 267 (R² to R⁵ are mainly primary hexyl groups) sold by Kalonite Chemical Co.; Hitec E 682 (R² to R⁵ are mainly primary hexyl groups) sold by Nippon Cooper Co., and Amoco 198 (R² to R⁵ are mainly primary butyl and amyl groups) sold by Amoco Chemical Co. may be used alone or in suitable combinations. It is then preferred that the proportion of the zinc dithiophosphate, in which the substituents R² to R⁵ are primary alkyl groups, is adjusted to at least 1/3, preferably at least 1/2.

The oxymolybdenum organophosphorodithioate sulfides are expressed in terms of the following formula:
wherein R⁶ and R⁷ may be identical or different, and stand for an alkyl, cycloalkyl, aryl or alkylaryl group having 1 to 30 carbon atoms, and x and y are a positive interger satisfying x + y = 4. The oxymolybdenum organophosphorodithioate sulfides may be prepared by the process disclosed in, e.g., JP-B-44-27366. By way of example, reference may be made to oxymolybdenum diisopropylphosphorodithioate sulfide, oxymolybdenum diisobutylphosphorodithioate sulfide, oxymolybdenum di-(2-ethylhexyl)phosphorodithioate sulfide, oxymolybdenum di-(p-tertiary butylphenyl)phosphorodithioate sulfide and oxymolybdenum di(nonylphenyl)phosphorodithioate sulfide.

More preferably, the phosphoric and phosphorous compounds are expressed in terms of the following formulae [III] or [IV]:
wherein R⁸, R⁹ and R¹⁰ may be identical or different, and stand for a hydrogen atom or an alkyl, aryl or alkyl-substituted aryl group having 4 to 30 carbon atoms.

By way of example, the phosphoric and phosphorous compounds may include phosphates and phosphites such as triphenyl phosphate, tricresyl phosphate, trixylenyl phosphate, tri(isopropylphenyl)phosphate, butyl acid phosphate, 2-ethylhexyl acid phosphate, lauryl acid phosphate, oleyl acid phosphate, stearyl acid phosphate, dibutyl hydrogen phosphite, dioctyl hydrogen phosphite, dilauryl hydrogen phosphite, dioleyl hydrogen phosphite and distearyl hydrogen phosphite, and amine salts such as laurylamine, oleylamine, coconut amine and tallow amine salts thereof.

The molybdenum alkyldithiocarbamates are expressed in terms of the following general formula [V]:
wherein R¹¹ and R¹² may be identical or different, and denote an alkyl group having 1 to 30 carbon atoms, which may or may not contain one oxygen atom therein, or a cycloalkyl, aryl or alkylaryl group having 1 to 30 carbon atoms, and x and y are a positive integer satisfying x + y = 4.

For the molybdenum alkyldithiocarbamates expressed in term of the general formula [V], use may be made of those disclosed in JP-B-49-6362 and 53-31646, and JP-A-56-61397 and 56-62894. By way of example, reference may be made to molybdenum diethyldithiocarbamate sulfide; molybdenum dibutyldithiocarbamate sulfide; molybdenum diamyldithiocarbamate sulfide; molybdenum di(2-ethylhexyl)dithiocarbamate sulfide; molybdenum dilauryldithiocabamate sulfide; molybdenum di(oleyl-linoeyl)dithiocarbamate sulfide; molybdenum dicyclohexyldithiocarbamate sulfide; molybdenum dinonylphenyldithiocarbamate sulfide; molybdenum 2-ethylhexyl (2-ethylhexyl-o-propoxy)dithiocarbamate sulfide; molybdenum 2-ethylhexyl (butyl-o-propoxy)dithiocarbamate sulfide and molybdenum 2-ethylhexyl (stearyl-o-propoxy)dithiocarbamate sulfide.

According to the present invention, the component (C) as mentioned above should be used in proportions of 0.1 to 10 weight %, preferably 0.5 to 10 weight % based on the total amount of the compositions. A proportion of the component (C) below 0.1 weight % is unpreferred due to an increase in wear losses, whilst a proportion of the component (C) exceeding 10 weight % is undesired due to increased corrosion and deteriorated stability.

The lubricating oil compositions for traction drive according to the present invention comprise the aforesaid components (A) to (C) and the below mentioned component (D) and, if required may contain various additives such as anti-foam agents, oiliness agents, friction modifier, corrosion inhibitors and fatigue life improvers, including rust inhibitor, anti-oxidants, pour-point depressants and viscosity index improvers.

Various rust preventing agent may be used. By way of example, reference may be made to calcium sulfonate, barium sulfonate and sodium sulfonate as well as alkyl or alkenyl succinates or their derivatives, alkylamines such as tri-n-butylamine, n-octylamine, tri-n-octylamine and cyclohexylamine, alkylamine or ammonium salts of carboxylic acids such as fatty acids or aromatic carboxylic acids having 6 to 20 carbon atoms and dibasic acids having 2 to 20 carbon atoms, or further condensed products of said carboxylic acids with amines. Among others, preference is given to calcium sulfonate or barium sulfonate.

As the anti-oxidants, use may be made to phenolic anti-oxidants such as 2,6-di-t-butyl-p-cresol and 4,4'-methylene-bis-(2,6-di-t-butylphenol) and amine base anti-oxidants such as dioctyldiphenylamine.

As the pour-point depressants or viscosity index improvers, reference is made to polymethacrylates having a number-average molecular weight of 10,000 to 100,000 in particular. Besides, olefin copolymers such as ethylene/propylene copolymers and styrene/propylene copolymers may be used to this end.

The lubricating oil compositions of the present invention are effectively used in winter and cold districts, since they have a high coefficient of traction and show a limited change in the coefficient of traction at low temperatures.

### Examples

The present invention will now be explained with reference to the examples and comparative examples.

### Preparation of (Base Oil)

1000 grams of tetralin (tetrahydronaphthalene) and 300 grams of concentrated sulfuric acid were put in a flask made of glass of 3-liter capacity, the interior of which was then cooled down to 0°C in ice bath. Under agitation, 400 grams of styrene were thereafter slowly added dropwise into the flask over 3 hours. Agitation was continued for further one hour to terminate the reaction. After the interruption of agitation, the reaction product was allowed to stand for the separation of an oily phase. The oily phase was washed with three portions each of 500 ml of an 1 N aqueous solution of sodium hydroxide and 500 ml of a saturated solution of sodium chloride, and was then dried over anhydrous sodium sulfate. After the removal of unreacted tetralin by distillation, distillation was carried out under reduced pressure to obtain 750 grams of a fraction having a boiling point of 135 to 148°C/22,66 Pa (0.17 mmHg). As a result of analysis, this fraction was found to be a mixture of 1-(1-tetralyl)-1-phenylethane with 1-(2-tetralyl)-1-phenylethane.

500 ml of the fraction was then put in an 1-liter autoclave, into which 50 grams of a 5% ruthenium/carbon catalyst were further added, for 4-hour hydrogenation under a hydrogen pressure 2.0 MPa of (20 kg/cm²) at a reaction temperature of 120°C. After cooling, the reaction liquid was filtered for the separation of the catalyst. After subsequent stripping-off of the light material out of the filtrate, the product was analysed. In consequence, it was ascertained that a hydrogenation degree of 99.9% higher was achieved, and the product was a mixture of 1-(1-decalyl)-1-cyclohexylethane with 1-(2-decalyl)-1-cyclohexylethane. The thus obtained mixture was found to have a specific gravity of 0.94 (15/4°C), a kinematic viscosity of 4,9 mm²/s (4.9 cSt) (100°C), a refraction index n$\frac{\text{20}}{\text{D}}$ of 1.5048 and a cis ratio of 88%.

### Example 1 and Comparative Example 1

The components specified in Table 1 were added to the base oil (the component A) obtained in the preparation example in the given proportions to obtain lubricating oil compositions, with which various testings were conducted by the following methods.

### Testing Methods

### Coefficient of Traction

The tests were carried out with a two-cylinder type rolling friction test machine. More specifically, while a cylinder A with a curvature (having a diameter of 52 mm and a radius of curvature of 10 mm) was in contact with a cylinder B with a plane (having a diameter of 52 mm) by 68670 N (7000 kgf), the cylinder A was rotated at a constant speed (1500 rpm) and the rotational speed of the cylinder B was increased from 1500 rpm. The coefficient of traction was then determined by measuring a traction force occurring between both cylinders at a slip rate of 5%.

The two cylinders were formed of bearing steel SUJ-2 and buffed on the surfaces to a surface roughness Rmax of 0.1 micrometer or less with alumina (0.03 micrometers), and were allowed to be in contact with each other at a Hertz contact pressure of 1098,7 N (112 kgf)/mm². The results are set out in Table 1.

### Anti-Wear Test

The four-ball tests according to ASTM D-4172 were conducted under the following conditions to determine wear losses (mm). The results are set out in Table 1.
Conditions: Revolutions per minute - 1,800 rpm.
Load - 294,3 N (30 kgf).
Time - 2 hours.
Oil Temperature - 120°C.

### Comparative Example 2

Example 1 was repeated, except that 4 weight % of polybutene (having a number-average molecular weight of 2,300) were used in place of the component (B). With the thus prepared lubricating oil composition, various tests were carried out. The results are set out in Table 1 and Figure 1.

**Table 1**

| No. | Composition (weight %) | | | | | | Wear Losses (mm) |
|---|---|---|---|---|---|---|---|
| | Component A *¹ | Component B *² | Component C *³ | | PMA *⁴ | Polybutene | |
| | | | I | II | | | |
| Example 1 | 93.0 | 4.0 | 0.5 | 0.5 | 2.0 | - | 0.50 |
| Comparative Example 1 | 93.0 | - | 0.5 | 0.5 | 6.0 | - | 0.55 |
| Comparative Example 2 | 93.0 | - | 0.5 | 0.5 | 2.0 | 4.0 | 0.52 |

| | | | | | | | |
|---|---|---|---|---|---|---|---|
| *1: Base oil obtained in the preparation example. | | | | | | | |
| *2: Ethylene-α-olefin copolymer having a number-average molecular weight of 2,600. | | | | | | | |
| *3: I ... Zinc dialkylthiophosphate wherein R² to R⁵ are primary hexyl groups. II ... Tricresyl phosphate. | | | | | | | |
| *4: Polymethacrylate having a number-average molecular weight of 40,000. | | | | | | | |

## Claims

1. A lubricating oil composition for traction drive, which comprises
(A) a base oil containing as the main component a saturated hydrocarbon or hydrocarbons having fused ring and/or nonfused ring,
(B) an ethylene-α-olefin copolymer having a number-average molecular weight of 800 to 8,000,
(C) an anti-wear agent, and
(D) a polymethacrylate having a number-average molecular weight of 10,000 to 100,000,
wherein the anti-wear agent is at least one selected from the group consisting of zinc dithiophosphate, oxymolybdenum organophosphorodithioate sulfide, phosphate, phosphite, amine salt of phosphate, amine salt of phosphite, molybdenum dialkyldithiocarbamate, mixtures of sulfurized fats and oils and posphates, mixtures of sulfurized fats and oils and phosphites, mixtures of sulfurized olefin and phosphates, mixtures of sulfurized olefin and phosphites, and the amine salts of the aforementioned mixtures.

2. A composition as claimed in claim 1, which contains 1 to 20 weight % of said ethylene-α-olefin copolymer and 0.1 to 10 weight % of said anti-wear agent.

3. A composition as claimed in claim 1, wherein said saturated hydrocarbon having fused ring includes decalyl group.

4. A composition as claimed in claim 1, wherein said saturated hydrocarbon having nonfused ring includes cyclohexyl group.

5. A composition as claimed in claim 1, wherein the ethylene-α-olefin copolymer have a number-average molecular weight of 1,000 to 5,000.

6. A composition as claimed in claim 1, wherein the ethylene-α-olefin copolymer have a number-average molecular weight of 2,000 to 4,000.

7. A composition as claimed in claim 1, wherein the ethylene content of the ethylene-α-olefin copolymer is 30 to 80 mol %.

## Patentansprüche

1. Schmierölzusammensetzung für Traktionsantrieb, umfassend:
(A) ein Grundöl, das als Hauptkomponente einen gesättigten Kohlenwasserstoff oder Kohlenwasserstoffe mit kondensiertem Ring und/oder nichtkondensiertem Ring enthält,
(B) ein Ethylen-α-Olefin-Copolymer mit einem mittleren (Zahlenmittel) Molekulargewicht von 800 bis 8 000,
(C) ein Antiverschleißmittel, und
(D) ein Polymethacrylat mit einem mittleren (Zahlenmittel) Molekulargewicht von 10 000 bis 100000,
worin das Antiverschleißmittel mindestens eines ausgewählt aus der Gruppe bestehend aus Zinkdithiophosphat, Oxymolybdän-Organophosphordithioatsulfid, Phosphat, Phosphit, Aminsalz von Phosphat, Aminsalz von Phosphit, Molybdändialkyldithiocarbamat, Gemischen von geschwefelten Fetten und Ölen und Phosphaten, Gemischen von geschwefelten Fetten und Ölen und Phosphiten, Gemischen von geschwefelten Olefinen und Phosphaten, Gemischen von geschwefelten Olefinen und Phosphiten und den Aminsalzen der zuvor genannten Mischungen ist.

2. Zusammensetzung nach Anspruch 1, die 1 bis 20 Gew.% des Ethylen-α-Olefin-Copolymeren und 0,1 bis 10 Gew.% des Antiverschleißmittels enthält.

3. Zusammensetzung nach Anspruch 1, worin der gesättigte Kohlenwasserstoff mit kondensiertem Ring eine Decalyl-Gruppe umfaßt.

4. Zusammensetzung nach Anspruch 1, worin der gesättigte Kohlenwasserstoff mit nichtkondensiertem Ring eine Cyclohexyl-Gruppe umfaßt.

5. Zusammensetzung nach Anspruch 1, worin das Ethylen-α-Olefin-Copolymer ein mittleres (Zahlenmittel) Molekulargewicht von 1 000 bis 5 000 aufweist.

6. Zusammensetzung nach Anspruch 1, worin das Ethylen-α-Olefin-Copolymer ein mittleres (Zahlenmittel) Molekulargewicht von 2 000 bis 4 000 aufweist.

7. Zusammensetzung nach Anspruch 1, worin der Ethylengehalt des Ethylen-α-Olefin-Copolymers 30 bis 80 Mol.% beträgt.

## Revendications

1. Composition d'huile lubrifiante pour entraînement par traction, qui comprend
(A) une huile de base contenant, comme principal constituant, un hydrocarbure saturé ou des hydrocarbures ayant un cycle condensé et/ou un cycle non condensé,
(B) un copolymère éthylène-α-oléfine ayant un poids moléculaire moyen en nombre de 800 à 8000,
(C) un agent anti-usure, et
(D) un polyméthacrylate ayant un poids moléculaire moyen en nombre de 10 000 à 100 000,
dans laquelle l'agent anti-usure est au moins une substance choisie dans le groupe formé par le dithiophosphate de zinc, un sulfure d'organophosphorodithioate d'oxymolybdène, un phosphate, un phosphite, un sel d'amine de phosphate, un sel d'amine de phosphite, un dialkyldithiocarbamate de molybdène, des mélanges de graisses et huiles sulfurées et de phosphates, des mélanges de graisses et huiles sulfurées et de phosphites, des mélanges d'oléfine sulfurée et de phosphates, des mélanges d'oléfine sulfurée et de phosphites, et les sels d'amine des mélanges susmentionnés.

2. Composition selon la revendication 1, qui contient 1 à 20 % en poids dudit copolymère éthylène-α-oléfine et 0,1 à 10 % en poids dudit agent anti-usure.

3. Composition selon la revendication 1, dans laquelle ledit hydrocarbure saturé ayant un cycle condensé comprend un groupe décalyle.

4. Composition selon la revendication 1, dans laquelle ledit hydrocarbure saturé ayant un cycle non condensé comprend un groupe cyclohexyle.

5. Composition selon la revendication 1, dans laquelle le copolymère éthylène-α-oléfine a un poids moléculaire moyen en nombre de 1000 à 5000.

6. Composition selon la revendication 1, dans laquelle le copolymère éthylène-α-oléfine a un poids moléculaire moyen en nombre de 2000 à 4000.

7. Composition selon la revendication 1, dans laquelle la teneur en éthylène du copolymère éthylène-α-oléfine est de 30 à 80 moles %.
